

## UNITED STATES PATENT OFFICE.

EUGEN SCHÜRER, OF COLOGNE-MULHEIM, GERMANY, ASSIGNOR TO FELTEN AND  
GUILLAUME CARLSWERK ACTIEN GESELLSCHAFT, OF COLOGNE-MULHEIM, GERMANY.

### MAGNETIZABLE MATERIAL.

No Drawing. Application filed August 13, 1925, Serial No. 50,143, and in Germany August 30, 1924.

Various alloys have hitherto been proposed which after suitable heat treatment show a high permeability and small losses in the case of small magnetizing forces. 5 Such alloys may for instance be used in the case of signalling lines in the construction of the cores of loading coils or in the case of a uniformly loaded conductor in the construction of the loading covering. Of the 10 already known alloys, the alloys the initial permeability of which may be made especially high by suitable annealing, have the drawback that when they are in a condition capable of being strongly magnetized, their 15 magnetic efficiency deteriorates under the influence of mechanical actions. For this reason special methods, some of which are complicated, have to be adopted in order to maintain these alloys in a state in which they 20 can be highly magnetized, for instance when they are to be used as loading material for uniformly loaded signalling lines.

According to the present invention the loading material of electric signalling conductors is made of an alloy which has favourable magnetic properties imparted to it 25 also by suitable heat treatment, which however has the advantage as compared with the known alloys that in the state in which it is capable of being strongly magnetized, it is not so sensitive to mechanical influences 30 as the alloys hitherto proposed for this purpose. It has been found by experiments that these requirements are fulfilled by an alloy 35 consisting of iron, aluminum and silicon, the

proportion of aluminum being greater than that of silicon and the latter being greater than 0.5%.

For the purpose of the present invention it has been found suitable to use an alloy 40 containing in addition to iron 1% of aluminum and about 0.7% of silicon.

The alloy proposed according to the present invention is known per se. However, the magnetic properties of this alloy in the case 45 of weak magnetic fields have not yet been investigated with respect to the requirements in signalling conductors. The special advantages of these alloys as compared with the alloys hitherto used when employed as loading 50 material for electric signalling conductors have not been known and these alloys have not hitherto been used for the purpose of the present invention.

What I claim is:—

1. A loaded signalling conductor the loading material of which consists of an alloy of iron, aluminum and silicon in which the proportion of aluminium is greater than that of silicon and the latter is not less than 55 0.5%.

2. A loading signalling conductor the loading material of which consists of an alloy of iron, aluminium and silicon in which the proportion of aluminium is 1% and that of silicon 0.7%.

In testimony whereof I have signed my name to this specification.

EUGEN SCHÜRER.